

March 14, 1939.

H. R. MINOR

2,150,287

SPONGE RUBBER BODY OF DIFFERENT DENSITIES

Original Filed May 16, 1936



FIG 1



FIG 4



FIG 2



FIG 5



FIG 3

INVENTOR.  
HENRY R. MINOR

BY *Henry R. Minor*  
ATTORNEYS.

## UNITED STATES PATENT OFFICE

2,150,287

SPONGE RUBBER BODY OF DIFFERENT  
DENSITIES

Henry R. Minor, Dayton, Ohio, assignor to Industrial Process Corporation, Dayton, Ohio, a corporation of New York

Original application May 16, 1936, Serial No. 80,191. Divided and this application December 21, 1936, Serial No. 116,959

## 1 Claim. (Cl. 18—53)

The object of my invention is to provide sponge rubber of different densities and of different strengths in different areas.

My invention particularly relates to seat cushions and the adaptation of the seat cushion in its shape to the configuration of the body resting upon it and in the density of its structure according to the place or places on which the greater weight of the person is applied.

It is a particular object of my invention to provide a sponge rubber seat cushion having areas of greater density where the greater weight is applied and to combine with this arrangement a seat cushion having a proper configuration for the reception of the weight of the body and the form of the body.

It is a further object to provide a method of loading a mold for forming such a seat cushion of sponge rubber.

This application is a division of my application Serial No. 80,191, filed May 16, 1936.

Referring to the drawing:

Figure 1 is a top plan view of the cushion.

Figure 2 is a side elevation thereof.

Figure 3 is a section on the line 3—3 of Figure 1 looking in the direction of the arrows.

Figure 4 is a top plan view of the mold partially loaded.

Figure 5 is a section on the line 5—5 of Figure 4 looking in the direction of the arrows.

Referring to the drawing in detail, I represents a sponge rubber seat cushion which may be either of a continuous body of sponge rubber of different densities and different areas, as at 2 and 3, or it may be formed of a seat portion 4 and vertical members 5 forming tubular areas 6 of different portions of the structure of greater density than others. The latter method is the preferred method of manufacturing this cushion.

If desired, the surface of the cushion may be formed with depressions 7 and the elevated areas 8 in order to provide a shaped surface for the reception of the body of the person sitting upon the cushion. Such depressed areas are ovoid in shape, as indicated in Figure 3.

In the manufacture of such a cushion, I prefer to use a sheet metal mold having side walls, top and bottom of sheet metal designated 9 with a plurality of open-ended tubes 10 extending into the interior of the mold. The tops of these tubes are closed as at 11 with the exception of a few perforations 12.

These tubes are staggered with respect to one another and arranged in rows. Between the rows are inserted in a vertical position the rubber

stock sheets 13 which are turned horizontally over the tops of the tubes as at 14 with their edges 15 overlapping the next adjacent portion 14 of the strip.

When it is desired to provide areas of greater density, either the stock sheets thus inserted may be made of a material as hereinafter described of greater density or additional sheets 16 may be inserted of the same or greater density than the adjacent sheets of stock. These sheets 16 will be of lesser length and will be confined to the particular area which it is desired to make of denser material to form the areas 2.

When the stock is thus arranged, the mold is closed and placed in a vulcanizer for vulcanization and curing in accordance with the practices outlined in my co-pending application Serial No. 59,625, filed January 17, 1936.

My process consists broadly of arranging the stock on edge with a portion horizontally disposed overlapping the next adjacent strip of stock; and of impregnating the stock with carbon dioxide gas under pressure; and thereafter applying the necessary heat as described in my co-pending application to bring about curing and vulcanization of the sponge rubber stock in sponge condition and of regulating that sponge as to its character and nature by the regulation of the escape of the carbon dioxide gas.

For instance, I find I am enabled to bring the pressure of impregnation up to 140 pounds to a square inch and gradually decrease it to zero while using a temperature as indicated.

When it is desired to make the stock of rubber denser in other areas, I have found such expedients as loading with clay, whiting and blanc fix, and even increasing the proportion of carbon black, a satisfactory means of increasing the density of the stock. Any of the well known methods of increasing the density of stock may be employed. Those I mention are merely typical.

It is understood that where the term "different densities" is used there is meant not only the change in mass per unit volume but also those changes in physical properties resulting in increased strength, resilience and resistance to deflection as may be obtained by the skillful compounder.

It will be understood that I desire to comprehend within my invention such modifications as come within the scope of my claim and my invention.

Having thus fully described my invention, what I claim as new and desire to secure by Letters Patent, is:

In a method of forming a homogeneous sponge rubber body comprising sections of varying densities, arranging stock rubber sheets of different physical properties in overlapping position with horizontal and vertical portions enclosing mold projections with the vertical portions of the stock arranged between the mold projections; enclosing the mold in an atmosphere of carbon dioxide gas

under pressure; and so regulating the temperature to which the stock and mold are subjected and the rate of escape of the carbon dioxide gas that a homogeneous body of sponge rubber of predetermined configuration having certain integral sections of different physical properties and densities is formed. 5

HENRY R. MINOR.